

## UNITED STATES PATENT OFFICE.

OSCAR TETENS, OF OERLINGHAUSEN LIPPE, GERMANY.

## PROCESS FOR THE PRODUCTION OF UNSINTERED BINDING MEANS OF OIL SHALE AND LIMESTONE AND THE LIKE.

No Drawing. Original application filed January 26, 1924, Serial No. 688,831. Patent No. 1,536,165.

Filed in Germany May 21, 1922. Divided and this application filed December 29, 1924. Serial No. 758,774.

The technical exploitation of the oil-shale has given certain practical results especially at the present time. Oil-shale is for instance utilized in such a manner that the residue of its gasification is worked up to artificial light stones. It has also been proposed to produce, by burning, cement, a sinter product, from the shale or from the residues after admixing the same with ground lime.

This invention relates also to this problem. When getting distillation products from shale and the burning of an unsintered hydraulic binding material is carried out simultaneously in the same operation, the heat produced by the combustion of the organic constituents of the shale, which have not been separated by distillation, is utilized to burn coke, lime-stone, chalky marl or the like which have been charged together with the raw shale. It has already been proposed to admix with the shale to be gasified small quantities of lime and chalky marl in order to be able to make after the burning of the shale ash building stones directly from the burnt material, the additions were however infinitesimally small while, according to my invention, they amount to 35-50% of the total charge and, if suitable chalky marl is used as addition, to an even higher percentage.

It has hitherto been believed that the calcining of lime-stone and the like by means of oil-shale were possible only with the aid of auxiliary fuel or with great quantities of shale. For this reason it is, according to another process of burning lime stone by means of oil-shale as a source of heat energy, necessary that the lime stone be charged into the kiln separately from the oil shale, that is traverses the kiln separately and is discharged from the kiln separately.

It has been discovered that these special measures are quite unnecessary and not only when oil-shale is used which possesses for instance a calorimetric value of from 2500 to 3500 calories, but even when oil shale is used the calorimetric value of which amounts to 800 to 1600 calories.

According to my invention the hot gases from combustion drive out the substances which are capable of being distilled out of the shale as it passes through the oven and

which they encounter above or beyond the combustion zone proper. The air required for the combustion flows, before it comes to combustion zone, through the hot zone of thoroughly burnt mixture. This air becomes heated by the residues and cools them according to the counter-current principle, so that the loss of heat is very low.

The practically complete combustion of the carbon of the shale-coke to carbon oxide is ensured, notwithstanding the high stock column used in the interset of the completest possible distillation of the volatile constituents of the oil-shale. The added lime-stone or calcareous marl acts upon decomposition by the heat, as heat absorbing material, preventing thus the formation of a too high temperature which would cause a decomposition of the carbon dioxide produced and therefore be unfavorable for the thorough combustion of the carbon to carbonic acid.

If the oven or shaft kiln is well insulated against the ambiant air almost the total heat liberated from the shale coke can be utilized.

As the shale residues, as lime- and aluminum silicate-containing materials, are opened at the burning they are capable of forming a valuable hydraulic binding material if ground with chalky lime or chalky marl or the like.

The process according to my invention can be applied also if lime-stone and shale are ground prior to the burning process and subsequently moulded to lumps.

When working according to the methods explained it is also possible to work in a part of the kilns on shale-lime or on Roman cement, as much lime-stone or chalky marl being charged as possible (for one part of shale up to 7 parts of the lime-containing substance according to the quality of the shale and to the composition of the lime-stone or the chalky marl). In the other part of the kilns the shale can be gasified in the commonly used manner without addition of lime. The gases produced can be used for instance for generating the energy required for the grinding of the binding material, the shale residue from this kiln being admixed with that from the other kilns, which is comparatively rich in lime, to be ground together with the same, the binding material

thus obtained is of better quality than it would otherwise be.

The process can be carried out in the shaft-kiln as well as in the revolving tubular kiln.

5 When shale- and lime-containing substances have hitherto been used to make binding material the purpose was to produce products similar to Portland cement or sintered products, the lime-containing substances were 10 added only in limited quantity. The lime-containing material was added only after the shale was distilled. In opposition hereto the shale is burnt, according to my invention, with a very high addition of lime and 15 worked in order to obtain an unsintered product.

I claim.

1. A process for the production of a hydraulic binding material from oil-shale and lime-containing material, which comprises 20 mixing the raw shale with lime-containing material capable of being calcined by the shale, distilling the mixture and recovering distillation products from the oil shale and 25 burning the mixture by the shale-coke obtained from such distillation in the same kiln and grinding the residues obtained by such burning.

2. A process for the production of a hydraulic binding material from oil-shale and lime-containing material, which comprises 30 grinding the raw shale together with at least thirty-five percent of lime-containing material, distilling the mixture and recovering 35 distillation products from the oil shale, burning the mixture without sintering in the same kiln, only by the shale coke distillation resi-

due, and grinding the residues obtained by such burning.

3. A process for the production of a hydraulic binding material from oil-shale and lime-containing material, which comprises 40 grinding the raw shale together with at least thirty-five per cent of lime containing material, molding the ground material to lumps, 45 distilling the lumps and recovering distillation products from the oil-shale, burning the mixture without sintering by the residual shale-coke in the same kiln and grinding the residue obtained by such burning. 50

4. A process for the production of a hydraulic binding material from oil-shale and lime containing material, which comprises 55 charging into one of a group of kilns raw shale mixed with a highest possible amount of lime-containing material capable of being calcined by the shale, distilling the mixture in a kiln and recovering distillation products from the oil-shale, burning the mixture in the same kiln without sintering by the shale-coke remaining from the distillation and distilling in another kiln the raw shale without 60 addition of lime-containing material, and grinding the residues from both kilns together to form hydraulic binding material. 65

5. The method of producing an unsintered hydraulic binding material which comprises mixing raw oil shale with at least thirty five percent calcareous material, distilling the mixture and simultaneously calcining the 70 material by the shale coke in the same kiln.

In testimony that I claim the foregoing as my invention, I have signed my name.

OSCAR TETENS.